

# UNITED STATES PATENT OFFICE.

DANIEL M. SORENSEN, OF TORONTO, ONTARIO, CANADA, ASSIGNOR TO EDSON L. CANNON, OF CLEVELAND HEIGHTS, OHIO.

## PROCESS OF TREATING BRAKE BANDS OF PLANETARY TRANSMISSIONS.

1,414,311.

Specification of Letters Patent. Patented Apr. 25, 1922.

No Drawing.

Application filed March 25, 1922. Serial No. 546,543.

To all whom it may concern:

Be it known that I, DANIEL M. SORENSEN, a subject of the King of Great Britain, residing at Toronto, in the county of York,

5 Province of Ontario, Dominion of Canada, have invented certain new and useful Improvements in a Process of Treating Brake Bands of Planetary Transmissions, of which the following is a specification.

10 This invention relates to a process for preventing the slipping or "chattering" of the speed or brake bands of the planetary transmissions of certain automobiles and is a continuation in part of my application No.

15 483,997, filed July 11, 1921.

As is well known to those familiar with the operation of such bands, the lubricants ordinarily employed therewith will, under the influence of the heat of the motor and 20 that due to the friction, produce a carbon residue which will form a hard glazed deposit upon the bands and their cooperating braking surfaces. The presence of this hard glazed deposit causes the brake bands, when 25 applied, alternately to grip, and to slip upon, the cooperating surfaces, producing what is known to the trade as the "chattering" of the bands.

In the practice of my invention I apply 30 to and between the brake bands and their cooperating surfaces or drums a lubricating compound produced as follows:

For a base for such lubricant, I employ an ordinary neutral mineral oil (such as defined in vol. 2 of The American Petroleum Industry, by Bacon & Hamor, published by McGraw-Hill Book Company, Inc., at New York in 1916) having a body varying in viscosity from 200° to 300°, Saybolt, at 35 100° F. To such base, I add, preferably about five per cent and not more than ten per cent, in quantity of a soap produced by saponifying fish, vegetable, or animal oil with ammonia or other appropriate alkali 40 45 and heating the soap to liquefy the same and render it miscible with such base.

The compound thus produced is not in-

juriously affected by the heat incidental to the operation of the motor and of the brake bands and will not produce an amount of 50 carbon sufficient to form the hard glazed deposit referred to and thereby prevent the smooth operation of such bands. On the other hand, it creates a soft film or surface 55 ing which acts as a cushion between the interengageable surfaces and prevents the alternate gripping and slipping, or "chattering" action.

Having described my invention, what I claim is:

1. The process of treating the brake bands of planetary transmissions to prevent the chattering thereof which consists in applying to and between such bands and their cooperating parts a lubricant comprising a 65 base of neutral mineral oil having a soap mingled therewith.

2. The process of treating the brake bands of planetary transmissions to prevent the chattering thereof which consists in applying to and between such bands and their cooperating parts a lubricant comprising a base of mineral oil having a viscosity of 70 from 200° to 300° and having a soap mingled therewith.

3. The process of treating the brake bands of planetary transmissions to prevent the chattering thereof which consists in applying to and between such bands and their cooperating parts a lubricant comprising a 80 base of mineral oil having a viscosity of from 200° to 300° and having mingled therewith not materially more than ten per cent of a soap.

4. The process of treating the brake bands of planetary transmissions to prevent the chattering thereof which consists in applying to and between such bands and their cooperating parts a lubricant comprising a 85 base of lubricating oil having a soap mingled therewith.

In testimony whereof, I affix my signature.

DANIEL M. SORENSEN.